

# UNITED STATES PATENT OFFICE.

GEORGE A. COLEHAMER, OF READING, PENNSYLVANIA.

## LUBRICATING COMPOUND.

Specification forming part of Letters Patent No. **11,359**, dated July 25, 1854.

*To all whom it may concern:*

Be it known that I, GEORGE A. COLEHAMER, of the city of Reading, in the county Berks and State of Pennsylvania, have discovered a new and useful composition of matter which is applicable as a substitute for sperm or other oils used for lubricating purposes; and I hereby declare that the following is a full, clear, and exact description of the manner of compounding and using the same.

This lubricating compound consists in the mixture of a fixed or vegetable oil—such as linseed-oil, olive, or other vegetable oil—with the crude article known in commerce as “rosin-oil and gum of camphor,” which may be mixed in various proportions. I have, however, found the following proportions of the ingredients to answer very well in the manufacture of the lubricating compound, viz: to make one gallon of my compound I take nine-sixteenths part of raw linseed-oil, seven-sixteenths of rosin-oil, and twelve pennyweights of gum-camphor, which ingredients, when well mixed, do then form a lubricating compound and fit for immediate use.

Some of the ingredients used in above-described compound may be replaced by others possessing similar properties—as, for instance,

instead of raw linseed-oil another vegetable oil might be used, such as rape-seed and other fixed oils—and so with the other ingredients, so that the compound would not be essentially changed in its character by substitutions or replacements. I do therefore not intend to limit myself to the precise ingredients above enumerated, but contemplate varying both the articles themselves and the proportions in which they are combined as economy in their cost or adaptation to particular purposes or other circumstances may render expedient.

Having thus described the manner in which I manufacture my lubricating compound, what I claim therein as new, and desire to secure by Letters Patent, is—

The combination of nine-sixteenths of a gallon of raw linseed-oil, seven-sixteenths of a gallon of rosin-oil, and twelve pennyweights of gum-camphor for a lubricator.

In testimony whereof I have hereunto set my hand and seal this 20th day of June, A. D. 1854.

G. A. COLEHAMER. [L. s.]

In presence of—

J. B. WANNER,  
P. H. FOLGER, 2d.